

May 10, 1927.

1,627,971

G. L. HERTZ

## MANUFACTURE OF VERY THIN WIRES

Filed April 22, 1925



INVENTOR.

G. L. HERTZ,

BY

L. T. & J. F. Brandenburg,  
ATTORNEYS.

Patented May 10, 1927.

1,627,971

# UNITED STATES PATENT OFFICE.

GUSTAV LUDWIG HERTZ, OF EINDHOVEN, NETHERLANDS, ASSIGNOR TO N. V.  
PHILIPS' GLOEILAMPENFABRIEKEN, OF EINDHOVEN, NETHERLANDS.

## MANUFACTURE OF VERY THIN WIRES.

Application filed April 22, 1925, Serial No. 25,164, and in the Netherlands June 18, 1924.

This invention relates to a process for the manufacture of very thin wires, more particularly of wires having a diameter of the order of some microns. In practice thin wires such as metal wires can frequently be made by means of a drawing process. According to such a process the diameter of little rods or thicker wires can be reduced by means of drawing dies. These drawing dies may consist, for example, of diamond through which a hole is bored corresponding to the diameter of the wire one wishes to manufacture. With the aid of drawing dies it is impossible, however, to draw wires of a very small diameter, because such wires break during the drawing process. The invention has for its object to provide a process according to which very thin wires can be easily produced without the use of drawing dies.

According to the invention the process for the manufacture of very thin wires consists in connecting wires of larger diameter as a cathode in a glow discharge at such a current density that disintegration of the cathode occurs.

It is known that in a glow discharge disintegration of the cathode occurs if the current density exceeds a certain value. In this case the potential drop at the cathode is greater than the normal cathode drop.

It has been found that by establishing for a considerable time a glow discharge of sufficiently high current density between the wire which is to be made thinner and which for this purpose is connected as cathode, and an auxiliary anode, the diameter of the cathode wire decreases and that in this manner wires can be made having a diameter of 1 micron or even less.

It is perhaps not unnecessary to observe that it is impossible to manufacture thin wires from wires of larger diameter by causing the latter to volatilize at a higher temperature. Volatilization is an unstable process, for an incandescent wire has the highest temperature in the thinnest places so that the volatilization is strongest there where the wire is thinnest. It is obvious that this circumstance leads to breakage of the wire. Disintegration, on the other hand, is a stable process, in which the phenomena occurring during volatilization do not present themselves and which permits the manufacture of thin wires having a diameter

which is practically equal over the whole length.

The process according to the invention is extremely suitable for the manufacture of very thin single crystal wires. The known processes for the manufacture of single crystal wires do not permit the manufacture of these wires with a diameter which is less than 10 microns, the drawing of thicker single crystal wires to a smaller diameter being impossible without the wire losing thereby its single crystal structure. The process according to the invention can be applied to all single crystal wires; by way of example may be mentioned: tin, zinc, tungsten, bismuth, cadmium, thallium lead, etc.

The invention will be described in detail and will be more clearly understood with reference to a mode of realization and to a figure representing the apparatus with which the process can be realized.

In the figure a tungsten wire 2 having a length of 2 decimetres and a diameter of 50 microns and from which one wants to manufacture a very thin wire, is sealed at 3 and 4 into a glass bulb 1, having a diameter of 6 centimetres. Besides, a second wire 5, for example of nickel, is sealed into the bulb at 6 and 7. The wire 2, the ends of which are electrically connected to each other, is connected to the wire 5 via a potentiometer in which a source of current having a tension of 500 volts is indicated by 8 and a regulable resistance by 9, via a resistance 10 of 10,000 ohms and a galvanometer 11 which permits to read 0.1 milliampere. The bulb 1 is filled with argon of a pressure of 0.2 millimetres of mercury. By so adjusting the sliding contact on the resistance 9 that the galvanometer indicates a current of 1 milliampere, the current density will be sufficiently great to cause the cathode to disintegrate.

During the disintegrating process the thickness of the cathode wire can be tested by measuring the resistance of said wire. If the disintegrating process is continued until the resistance of the wire 2 is increased to about the twentyfold amount of the resistance of the original wire, it appears that the cathode wire has a diameter of but some microns. It is however possible to continue the process still further and to obtain thus wires having an even considerably smaller

diameter. When the diameter of the cathode wire has been sufficiently reduced, the wire may be removed from the bulb 1 by breaking the seals 2 and 3.

5 Wires manufactured in accordance with this process are very suitable for the use as resistance thermometers in string galvanometers according to Einthoven and other apparatus in which it is desirable to utilize  
10 very thin wires.

What I claim is:

1. A process for the manufacture of very

thin wires, characterized in that wires of larger diameter are connected as cathode in a glow discharge at such a current density that disintegration of the cathode occurs.

2. Single crystal wires having a diameter of less than 10 microns.

In testimony whereof I affix my signature, at the city of Eindhoven this 4th day of April, A. D. 1925.

GUSTAV LUDWIG HERTZ.